

## UNITED STATES PATENT OFFICE

RENÉ PICARD, OF PARIS, FRANCE, ASSIGNOR TO SOCIETE ALSA IN BASEL, A CORPORATION OF SWITZERLAND

## ARTIFICIAL HOLLOW THREAD MANUFACTURING PROCESS

No Drawing. Application filed April 27, 1928, Serial No. 273,426, and in Germany April 30, 1927.

Persons skilled in the art are aware of the prior artificial hollow thread manufacturing processes or methods (patents Brandenberger No. 1,394,270, Rousset No. 1,487,807 and Brandenberger No. 1,544,631) including those wherein viscose having a carbonate dissolved therein is spun in an acid bath.

The spaces or voids produced in the filaments may be formed of adjoined bubbles separated by cross partitions. Such threads generally maintain their hollow spaces on account of the rigidity imparted thereto by their cross-partitions.

In other instances, the hollow threads have only a few partitions, or none at all, whereby, and particularly in the case of fine filaments, the outer walls will close in or collapse, somewhat after the manner of a collapsed rubber tube. These threads generally have less covering power than the cross-partitioned ones.

This invention contemplates the manufacturing of hollow threads endowed with a higher covering power, even where the spaces are partitionless.

The process or method constituting the invention is characterized by the fact that acid coagulating baths containing a high proportion of zinc sulphate (practically over 6%) are used.

In the coagulating bath containing zinc sulphate hitherto used in artificial silk manufacturing practice, the zinc sulphate proportion is about 1% and, according to DRP Patent No. 260,479, should not exceed 5% in order to avoid noxiousness. On the other hand, English patent discloses baths for hollow thread manufacturing containing zinc sulphate up to 4% and 5%.

Said patents do not cover the use of a relatively large proportion of zinc sulphate in coagulating baths nor do they recognize the remarkable effect arising therefrom as to the covering power of threads so obtained.

The influence of high zinc sulphate proportions on coagulation is such that when the bath contains nothing but sulphuric acid and sulphate of zinc, the latter in a 30% proportion, there is obtained a hollow thread which—weight equal—bulks far more than any obtained by hitherto known methods.

In addition to sulphuric acid and zinc sulphate, the coagulating bath may also contain sulphate of soda or other coagulating salts, or such products as glucose, which have been found advantageous in the artificial silk industry. 55

*Practical example.*—In a normal viscose containing: cellulose 7%, and alkali 6, 5%, 4% of carbonate of soda is dissolved. The solution is then allowed to ripen or mature 60 until it possesses a salt point of 10 (an explanation of "salt point" is given in French Patent No. 577,369, dated August 13th, 1923), at which time it is spun in a coagulating bath composed as follows:

|                  | Grams per liter |
|------------------|-----------------|
| Sulphuric acid   | 120             |
| Zinc sulphate    | 220             |
| Sulphate of soda | 40 70           |

under the conditions required to obtain a unit strand of 3, 7 dwt.

The thread is then finished according to the usual artificial silk treatment.

Having now particularly ascertained and described the nature of my said invention as well as the manner in which the same is to be performed, I declare that what I claim is:

1. In a process of producing hollow artificial silk threads the step which comprises spinning the viscose solution in an acid coagulating bath containing zinc sulphate in excess of 6%. 80

2. In a method of producing hollow artificial silk threads the step which comprises spinning the viscose solution in an acid coagulating bath containing 6% to 30% of zinc sulphate. 85

3. In a process of producing hollow artificial silk threads the step which comprises spinning the viscose solution in a coagulating bath comprising 120 grams per liter of sulphuric acid, 220 grams per liter of zinc sulphate and 40 grams per liter of sodium sulphate. 90 95

In testimony whereof I affix my signature.

RENÉ PICARD.